

## 1

3,234,025

**PREVENTION OF DYE-DIFFUSION IN PHOTOGRAPHIC IMAGE BEARING COLLOID LAYERS**  
 Albert Emiel Van Hoof, Berchem-Antwerp, and René Maurice Hart, Wilrijk-Antwerp, Belgium, assignors to Gevaert Photo-Producent N.V., Mortsel-Antwerp, Belgium, a Belgian company

No Drawing. Filed Aug. 2, 1960, Ser. No. 46,879  
 Claims priority, application Belgium, Aug. 4, 1959,  
 581,344, Patent 39,134  
 2 Claims. (Cl. 96—95)

The present invention relates to the prevention of diffusion of dyes in colloid layers, in particular to a new process for the preparation of mordants for acid dyes and for their application, especially for the manufacture of colour images according to the hydrotype process particularly on an improved cinematographic blank film on which colour images are printed according to the hydrotype process.

For the manufacture of colour films according to the hydrotype process, a film support bearing a relief image obtained in a photographic way is used as starting material. Said relief image consists of a colloid, in most cases gelatin. The whole is referred to as a matrix or matrix film. This matrix is immersed in a dye-solution and brought into close contact with another film which is referred to as a blank or blank film.

Because of the contact between the dyed matrix film and the blank film, the dye of the image relief of the matrix diffuses to the hydrophilic colloid layer on the blank film on which a monochrome image is formed. In the same way a second monochrome print is obtained, etc.

This dye-transfer process can thus be repeated to such an extent that many monochrome prints can be made with one single matrix. Also multicolour images can be obtained by immersing a second matrix in another appropriate dye-solution and by transferring the dye to a blank on which already a monochrome image has previously been printed. This process can be continued with other matrices and dyes as described in Colour Cinematography, A. Cornwell-Clyve, 3rd ed., 1951, pages 451—474.

Said process, however, meets with the great disadvantage that the definition of the colour image is poor, due to the lateral diffusion of the dyes in the hydrophilic colloid layer of the blank film. This lack of definition is a serious drawback when the colour image is enlarged to great dimensions e.g. during cinematographical projection on a screen.

It is already known to incorporate into the hydrophilic colloid layer of the blank film mordants which precipitate the dye so as to prevent this dye from lateral diffusion. In consequence thereof colour images are obtained showing a much better definition.

It is also known from U.S. specification 2,548,564 that addition polymers prepared from substituted vinyl azines and vinyl azoles containing quaternary ammonium groups can be used as mordants for soluble acid dyes in photographic layers.

For the same purpose it is known from the U.S. Patent 2,675,316 to use polyvinyl dialkylamines consisting of structural units, either quaternary or not quaternary, of the type



## 2

wherein  $\text{R}_1$  and  $\text{R}_2$  each represents an alkyl group or together represent the atoms necessary to close an alicyclic or a heterocyclic ring.

It is further known from the Belgian specification 540,976 to incorporate polyvinyl amines into blank films as mordants for acid dyes.

Finally it is known from the British specification 830,189 to use as mordants for acid dyes hydrolyzed or solvolyzed derivatives of polymers containing structural units of the type:



15 wherein  $\text{R}$  represents an alkyl or aralkyl radical.

Among the many disadvantages of the mordants proposed hereinbefore, the staining, also called matrix poisoning, of the matrix by these mordants has to be mentioned. Said matrix poisoning is caused in case the used mordant is not sufficiently fast to diffusion. In consequence thereof some of these mordants pass from the blank upon the matrix when both the films are in close contact with each other. When the matrix is reimmersed into the dye solution, the latter will not only adhere on the image relief but also precipitate on those areas where the matrix has been poisoned by the mordant. Consequently, besides the desired colour image a more or less uniform colour-fog is formed on a following colour print. This harmful colour-fog formation will be repeated and evidently increased during the production of further prints. Moreover other unspecified products of the blank may cause the staining of the matrix.

35 Although many means are known for preventing said matrix poisoning and the subsequent formation of colour fog resulting from this staining on the prints, they are either not effective or they complicate the process e.g. by necessitating the application of special addition layers in the matrix film.

40 A further disadvantage of some of the used mordants resides in the fact that they result in an insufficiently low colour absorption. By colour absorption is meant the maximum colour density obtainable in definite circumstances of time and temperature under which the dye-immersed matrix is brought into close contact with the blank. Said conditions are required by the apparatus ensuring the contact between the matrix and the blank film.

45 It is known from the Belgian patent specification 511, 50 to add high molecular nitrogen bases, their salts or their quaternary derivatives, which all are fast to diffusion, as mordants to photographic and reproduction material. In said patent polyethylene imine is cited by way of example for such mordants. This polymer effects a mordant action but it has too low a color absorption and furthermore causes matrix poisoning to a very high extent.

55 Now it has been found that the lateral diffusion of dyes in colloid layers and the diffusion of dyes out of colloid layers can be prevented by incorporating in said colloid layers reaction products of polyethylene imine and urea. The reaction products of polyethylene imine and urea are formed by reacting, whilst heating, a mixture which consists of polyethylene imine and urea.

60 Although polyethylene imine is referred to as a polymer consisting of a series of linearly bound



65 groups, recent investigations of a commercial product

have proved that polyethylene imine is composed of 30% of  $-\text{CH}_2-\text{CH}_2-\text{NH}_2$  units, 40% of



units and 30% of



units. The specific viscosity of polyethylene imine measured in a 1% aqueous solution amounts to 0.22. The ratio of the reacting amounts of polyethylene imine and urea may vary within defined limits. The most suitable mordants however are obtained by condensing 0.1 to 5 mols urea with 1 mol polyethylene imine.

The use of an excessive amount of urea reduces the mordant power of the polymer in such a way that the produced color image shows lack of definition. When urea is used in too small a quantity, the color absorption of the polymer is on the lower side. The structure of the polymers obtained is not exactly known, but it is admitted that the imino groups are partially substituted by the urea.

An advantage of the mordants according to the present invention resides in the possibility that the color absorption can be brought on a favorable level by modifying the composition of these mordants.

A further important advantage of the mordants according to the present invention is the absence of matrix staining.

Another advantage of these mordants is their applicability in colloid layers at pH-values of about 6 to 7 without involving too high an increase of viscosity as in the case of the application of the mordant polymers previously described in the prior art.

The blank film on which color images are printed according to the hydrotype method consists mainly of one or more layers of a hydrophilic colloid such as gelatin, polyvinyl alcohol, etc. coated on a film support. One of said composing colloid layers may be a silver halide emulsion layer.

The usual supports for the manufacture of the matrix film and the blank film in most cases are composed of cellulose derivatives, especially cellulose-esters, such as cellulose triacetate, cellulose acetobutyrate, cellulose propionate or even fully synthetic polymerization products or polycondensation products e.g. polyethylene glycol terephthalate, polycarbonates and polysulfonates.

Evidently the application of the polymers as mordants according to the present invention is not necessarily limited to the use as mordants in blanks for the production of prints according to the hydrotype process. These polymers can equally be applied to processes for the mordanting of acid dyes or of compounds with a relatively large anion, such as e.g. anti-static products, wetting agents, etc.

One of these further ways of application is e.g. to use, as filter layers, layers containing a hydrophilic colloid such as gelatin which comprises a mordant according to the present invention and an acid dye. Such filter layers are among others employed in an antistress layer or an intermediate layer e.g. in a multicolor film which is composed of different emulsion layers, or even in an antihalo layer. The new process can furthermore be applied in the preparation of pigmented layers such as pigmented paper. The polymers according to the present invention can also be used in the manufacture of photographic color material for rendering color couplers fast to diffusion. Detailed particulars regarding these special applications are disclosed in British patent specification 830,189.

#### PREPARATION 1

In a flask fitted with a stirrer and a condenser 19.8 g. of a 50% aqueous polyethylene-imine solution are added to 72 cm.<sup>3</sup> of water and 21.6 g. of urea. The mixture obtained is refluxed for 15 hrs. whereby ammonia is liberated. After cooling, 100 cm.<sup>3</sup> of acetone are added to the reaction mixture for precipitating the product thus

obtained. After decanting, the product is dissolved in 25 cm.<sup>3</sup> of distilled water, and precipitated again in an excess of a mixture consisting of equal parts of acetone and methanol. After decanting and drying, 13.8 g. of reaction product are obtained. Next 10 g. of this product are dissolved in 80 cm.<sup>3</sup> of distilled water, neutralized with strong hydrochloric acid and filled up to 110 g. with water.

#### PREPARATION 2

In a flask fitted with a condenser and a stirrer is brought a solution of 20.6 g. of polyethylene imine and 15 g. of urea dissolved in 220 cm.<sup>3</sup> of water. This reaction mixture is stirred and refluxed for 8 hrs. at 100° C. whereby ammonia is liberated. The polymer formed is purified by precipitation in acetone. After decanting the polymer is neutralized with hydrochloric acid. Finally water is added to obtain a 10% polymer solution.

#### PREPARATION 3

Analogously to preparation 2, 20.6 g. of polyethylene imine are dissolved in 220 cm.<sup>3</sup> of water and reacted with 30 g. of urea whilst ammonia is liberated. Then the polymer is purified and dissolved as described in preparation 2.

#### PREPARATION 4

500 cm.<sup>3</sup> of a 25% aqueous polyethylene imine solution and 250 cm.<sup>3</sup> of a 50% aqueous urea solution are mixed. This mixture is boiled for 2 hrs. in an open vessel whereby ammonia is liberated. The amount of evaporated water is regulated by filling up with boiling water. After cooling the reaction mixture is purified in the same way as in preparation 1 by precipitation in acetone.

The following examples illustrate the invention without limiting, however, the scope thereof.

#### Example 1

A layer-forming solution is made of the following composition:

|                                                         | Cm. <sup>3</sup> |
|---------------------------------------------------------|------------------|
| 8% aqueous gelatin solution                             | 1000             |
| 10% aqueous polymer solution according to preparation 3 | 100              |

With hydrochloric acid N the pH is brought to 4 and a solution is added composed of

|                                   |                    |
|-----------------------------------|--------------------|
| Saponin                           | g. 0.5             |
| 40% aqueous formaldehyde solution | cm. <sup>3</sup> 4 |

The resulting solution is coated onto a support of cellulose triacetate film provided with a subbing layer, solidified and dried; on the blank film thus obtained one or more color images can be printed according to the hydrotype process. When these images are cinematographically projected they show an enlarged image of good definition.

#### Example 2

A silver halide emulsion layer used for positive prints is applied to a support of cellulose triacetate film which is provided with a subbing layer. Onto this emulsion layer, a layer of following composition is coated:

|                                                            |                      |
|------------------------------------------------------------|----------------------|
| Gelatin                                                    | g. 50                |
| Water                                                      | cm. <sup>3</sup> 800 |
| 10% aqueous polymer solution according to preparation 4    | cm. <sup>3</sup> 100 |
| Water to 1000 cm. <sup>3</sup>                             |                      |
| Condensation product of iso-octylphenol and ethylene oxide | g. 0.2               |
| Glyoxal                                                    | cm. <sup>3</sup> 5   |

After solidifying and drying a sound track can photographically be applied to the film thus obtained. On the same film, three gelatin image reliefs can successively be printed, each of these reliefs having previously been immersed in an appropriate acid dyestuff solution, according to the method disclosed in "Colour Cinematography," Cornwell-Clyve, 3rd edition, 1951 pages 451-474, in order to obtain a multicolor image.

## 5

## Example 3

A solution A and a solution B respectively composed of:

|                                                           |                          |    |    |
|-----------------------------------------------------------|--------------------------|----|----|
| A gelatin                                                 | -----g--                 | 30 | 5  |
| Ponceau 2R (Color Index No. 16,150)                       | -----g--                 | 1  |    |
| Water to 1000 cm. <sup>3</sup> .                          |                          |    |    |
| B gelatin                                                 | -----g--                 | 30 |    |
| 10% aqueous polymer solution (according to preparation 2) | -----cm. <sup>3</sup> -- | 30 | 10 |
| Water to 1000 cm. <sup>3</sup> .                          |                          |    |    |

are formed together at 35° C. whilst thoroughly stirring. The resulting suspension of the insoluble complex of dye-stuff and mordant polymer is coated as a light filter layer onto a support of cellulose triacetate which is provided with a subbing layer. 15

## Example 4

Similarly to Example 2 pigmented gelatin sols can be prepared by changing the incorporated acid dyes. These 20 pigmented gelatin sols are coated onto a paper support to form a so-called pigmented paper which can be used for the production of colored images according to the processes known in the art (carbon, carbro).

We claim:

1. A photographic element comprising a support and a layer of gelatin on said support, said layer having dis-

## 6

tributed therein a substantially neutralized water-soluble condensation product obtained by heating in an aqueous medium a water-soluble polyethylene imine having a specific viscosity of 0.22 measured in a 1% aqueous solution and urea with the liberation of ammonia, said imine and urea being present in amounts providing a molar ratio of about 0.1-5:1 of urea to said imine.

2. The photographic element of claim 1 wherein said condensation product is attained by heating said aqueous medium containing said imine and urea at the boil for about 2-15 hours.

## References Cited by the Examiner

## UNITED STATES PATENTS

2,912,296 11/1959 Taube et al. ----- 260-2 X

## FOREIGN PATENTS

543,893 7/1957 Canada.

755,478 5/1956 Great Britain.

782,217 9/1957 Great Britain.

## OTHER REFERENCES

Wilfinger: "Das Papier" 2, pages 265-75 (1948).

25 NORMAN G. TORCHIN, Primary Examiner.

PHILIP E. MANGAN, Examiner.